

# UNITED STATES PATENT OFFICE.

JOSZYP MOSZYNSKI, OF PHILADELPHIA, PENNSYLVANIA.

## TANNING AND WATERPROOFING LEATHER.

1,157,952.

Specification of Letters Patent.

Patented Oct. 26, 1915.

No Drawing.

Application filed July 28, 1913. Serial No. 781,699.

*To all whom it may concern:*

Be it known that I, JOSZYP MOSZYNSKI, a subject of the Emperor of Russia, residing at Philadelphia, in the county of Philadelphia and State of Pennsylvania, have invented a new and useful Improvement in Tanning and Waterproofing Leather, of which the following is a specification.

This invention relates to the process of 10 tanning and waterproofing the leather in a short space of time and at less expense, making a soft pliable leather.

The ingredients used, and the method of using the same, follow:—Concentrated sodium sulfid  $\frac{1}{4}$  pound, 40 degrees barkometer test, lime  $\frac{1}{4}$  pound, 40 degrees barkometer test, chestnut extract 10 pounds, cutch extract 10 pounds, soda ash, oil of vitriol, oxalic acid, paraffin 1 pound, yellow wax 20 1 pound, fat suet 2 pounds.

In use, the hide is placed in cold water for one and one-half days, then immersed in a solution of concentrated sodium sulfid and lime, each testing 40 degrees, barkometer, 25 for three days at a heat of 110 degrees, Fahrenheit. The hide is then shaved and placed in clear cold water for twelve hours; removed and placed in a composition of cutch extract 10 pounds and chestnut extract 10 pounds and water to test 25 degrees, barkometer, each, from which it is removed and placed in a bath of vitriol oil at 30 30 35 40 45 50 30 degrees, barkometer, for three days, when it is placed in a bath composed of cutch extract and chestnut extract each testing 25 degrees, barkometer, for twelve days, increasing the strength of the bath every third day ten degrees, barkometer; remove and place in soda ash bath of 25 degrees, barkometer, at 126 degrees Fahrenheit, for 15 minutes, remove and place in vitriol oil at 30 degrees, barkometer, for five minutes at 130 degrees, Fahrenheit, then in clear cold water for one-half hour. It is then placed in the dry house for 5 days at a temperature of 145 degrees, Fahrenheit. The paraffin, one pound, yellow wax, one pound and fat suet, 2 pounds, are heated to 130 degrees, mixed thoroughly and brushed on the leather, after a thorough brushing it is placed in the dry house at a temperature of 110 degrees, for

ten hours. After thoroughly dry place in soda ash testing 25 degrees, barkometer, for 15 minutes at a temperature of 126 degrees, then place in vitriol oil testing 30 degrees, barkometer, at a temperature of 130 degrees, for 5 minutes, then in cold water for three hours when it is removed to the dryhouse, where it must remain for 12 hours, after which it is placed on the rolling machine; 60 after the first rolling brush over quickly with oxalic acid and again roll; after the second rolling it is placed in the dry-house for 12 hours, after which time it is ready for use. 65

By the use of the above method the hair is speedily and thoroughly loosened, and the hides cleaned from grease and other substances which would prevent them from being tanned quickly. The use of the other ingredients, as specified, results in a well tanned, water proof and preserved leather in a less period than formerly employed. 70

I claim:—

The process of tanning leather after the 75 hides have been depilated, the hide is immersed in a bath consisting of water, cutch extract 10 pounds, chestnut extract 10 pounds said bath to test 25 degrees barkometer, to be then immersed in a bath of 80 vitriol oil testing 30 degrees barkometer from which the leather is taken and placed in a bath composed of cutch extract and chestnut extract and water to test 25 degrees barkometer, the said bath being increased in 85 strength at determined times 10 degrees by the addition of the aforesaid extracts, then immersed in a soda ash bath testing 25 degrees at 126 degrees Fahrenheit for a determined period, when it is placed in vitriol 90 oil of 30 degrees barkometer, from the said bath to cold water for the specified time, and then dried, after which it is ready to be made waterproof.

In testimony whereof I affix my signature 95 in the presence of the subscribing witnesses.

JOSZYP MOSZYNSKI.

Witnesses:

W.M. MACDONALD,  
TUKUB LEWANDORK,  
KARMER RUTECKI.

Copies of this patent may be obtained for five cents each, by addressing the "Commissioner of Patents, Washington, D. C."